

## UNITED STATES PATENT OFFICE

2,089,293

## SAFETY PAPER

Clifford Paine and Jack Augustus Radley, Blackley, Manchester, England, assignors to Imperial Chemical Industries Limited, a corporation of Great Britain

No Drawing. Application August 5, 1935, Serial No. 34,839. In Great Britain August 8, 1934

17 Claims. (Cl. 91—67.95)

The present invention relates to the manufacture or preparation of improved safety papers, that is to say of papers mainly used for commercial and legal documents, cheques, bank notes, bonds and the like, the paper being so treated as to prevent writing or printing thereon from being successfully tampered with.

It is known to employ chemically treated papers for the prevention of tampering, the chemicals used for such treatment being selected so as to give visible stains in contact with inkeradicating agents. It has also been proposed to employ papers treated with fluorescent substances so that unauthorized alterations or the like, although not detectable in ordinary daylight, are made visible by inspecting the document under filtered ultra-violet light. In British specification 292,393 it is proposed to use for such treatment of paper a water-soluble fluorescent salt, namely the sodium salt of 2-naphthol-3:6-disulphonic acid. The fluorescent substance described in the said specification has the disadvantage that the surface fluorescence produced by it in the paper is susceptible to destruction by water alone. It is therefore possible for the "cheque raiser" or forger first to extract the fluorescent substance from the paper with water, make unauthorized alterations to the printed or written document and thereafter restore the document to its normal appearance by re-treating it with a suitable fluorescent aqueous solution. To overcome this disadvantage a further improvement was proposed in British specification 417,488 whereby the fluorescent agent incorporated in or applied to the paper was to be a water-insoluble compound, such as fluorine or acridine, in the form of a suspension.

There are, however, disadvantages in the use of water-insoluble fluorescent compounds for such purposes. In general it is necessary to use relatively large amounts of suspensions of such compounds in order to obtain the desired degree of fluorescence unless extremely highly dispersed suspensions are used. Such dispersions are troublesome to make, liable to be unstable, or flocculated by other chemicals used in the preparation or finishing of paper so that uniform incorporation or surface application is made difficult. We have found that the disadvantages of the known processes can be overcome by the use of certain fluorescent compounds as herein-after defined which are water-soluble but which, because of their strong affinity for cellulose, are extremely difficult to remove from papers to which they have been applied.

According to the present invention we incorporate into paper or apply superficially to it the free acid or a water-soluble salt of 4:4'-dibenzoylaminostilbene-2:2'-disulphonic acid (see Stobbe and Mallison, Ber. der deutschen Chem. Gesellschaft, 1913, 46, 1235) or a substitution derivative thereof. As substitution derivatives we may use, for example, 4:4'-di-p-aminobenzoylaminostilbene-2:2'-disulphonic acid, 4:4'-di-o-chlorobenzoylaminostilbene-2:2'-disulphonic acid, 4:4'-di-p-methylbenzoylaminostilbene-2:2'-disulphonic acid. The compounds for use according to the invention are readily made by reacting the appropriate aroyl halides with the sodium salt of 4:4'-diaminostilbene disulphonic acid in aqueous medium in the presence of a mineral acid binding agent, for example, sodium acetate or sodium carbonate.

The present invention may be carried into effect in a variety of ways. The said water-soluble fluorescent compounds as already mentioned have, although substantially colourless, a marked affinity for cellulose, for example paper pulp, on which they may be "dyed" by the methods customary in applying direct dyestuffs to cotton. By virtue of these properties the said compounds may be incorporated into the texture or felting of a paper during manufacture. Thus paper pulp may be "dyed" with the said fluorescent compounds prior to the formation of a paper or pulp so "dyed" may be applied superficially to a layer of "undyed" pulp during the manufacture of a paper. Alternatively, a pre-formed paper may be "dyed" by immersion in an aqueous solution of the said compounds. Where the invention is carried into effect by "dyeing" a pulp or paper it has been found that less than 0.5%, generally about 0.1% by weight of the fluorescent compound in relation to the weight of cellulose material to be "dyed" is sufficient to obtain satisfactory fluorescence. In another embodiment of the invention an aqueous solution of the said fluorescent compounds may be applied superficially to paper by spraying, brushing or printing.

Papers treated according to the invention fluoresce with a bluish hue when exposed to filtered ultraviolet radiations, whereas if subjected in parts to the action of ink bleaching chemicals such as calcium hypochlorite, permanganate, and oxalic acid or the like, or, provided a superficial coating of the stilbene derivative has been applied, if subjected to the action of an ink eraser, such localized treatment is immediately apparent under the ultraviolet lamp, the parts so treated ceasing to fluoresce and ap-

pearing dark against a bluish ground. Thus attempts to eradicate or alter writing on paper treated according to the invention are readily detected. Further, the fluorescent compounds used as indicators of such tampering are not readily removed from the safety papers by contact with water.

The following examples illustrate but do not limit the invention. The parts are by weight.

10

*Example 1*

A solution of 0.1% strength of p:p'-diamino-4:4'-dibenzoyldiamino-stilbene-2:2'-disulphonic acid sodium salt is applied to the surface of paper 15 at a convenient part of a paper machine by means of a water doctor or spray in the well known manner. The paper is dried as usual on the drying rolls which follow the said convenient part. If desired the stilbene sulphonic acid derivative can be applied to the paper pulp in the beater but since the whole body of the paper will then be impregnated with the sulphonic acid, it will not be so sensitive to surface erasures, but will be equally sensitive to bleaching chemicals 25 which penetrate through the paper.

*Example 2*

Sufficient of the same stilbene compound as used in Example 1 is added to a 2% solution of gelatine, glue or casein to make a 0.1% solution of the stilbene sulphonic acid derivative which is then applied to the surface of the paper by brushing, dipping, spraying or printing. Drying is effected in any convenient manner.

35 We claim:

1. The method of rendering paper and the like sensitive to ink eradicating chemicals which comprises incorporating therein a 4:4'-di-(benzoyl-amino) stilbene 2:2'-di-sulfonic acid compound.
- 40 2. The method of rendering paper and the like sensitive to ink eradicating chemicals which comprises incorporating therein an alkali metal salt of a 4:4'-di-(benzoyl-amino) stilbene 2:2'-disulfonic acid compound.
- 45 3. The method of rendering paper and the like sensitive to ink eradicating chemicals which comprises incorporating therein a 4:4'-di-(aminobenzoyl-amino) stilbene 2:2'-di-sulfonic acid compound.
- 50 4. The method of rendering paper and the like sensitive to ink eradicating chemicals which comprises incorporating therein an alkali metal salt

of a 4:4'-di-(benzoyl-amino) stilbene 2:2'-disulfonic acid.

5. The method of rendering paper and the like sensitive to ink eradicating chemicals which comprises incorporating therein an alkali metal salt 5 of a 4:4'-di-(aminobenzoyl-amino) stilbene 2:2'-disulfonic acid.

6. The method of rendering paper and the like sensitive to ink eradicating chemicals which comprises incorporating therein an alkali metal salt 10 of 4:4'-di-(p-amino-benzoyl-amino) stilbene 2:2'-disulfonic acid.

7. Paper and the like having incorporated therein a 4:4'-di-(benzoyl-amino) stilbene 2:2'-di-sulfonic acid compound. 15

8. Paper and the like having incorporated therein an alkali metal salt of a 4:4'-di-(benzoyl-amino) stilbene 2:2'-disulfonic acid compound.

9. Paper and the like having incorporated therein an alkali metal salt of a 4:4'-di-(amino-benzoyl-amino) stilbene 2:2'-disulfonic acid. 20

10. Paper and the like having incorporated therein an alkali metal salt of a 4:4'-di-(benzoyl-amino) stilbene 2:2'-disulfonic acid.

11. Paper and the like having incorporated 25 therein an alkali metal salt of 4:4'-di(p-amino-benzoyl-amino) stilbene 2:2'-disulfonic acid.

12. The method of rendering paper and the like sensitive to ink eradicating chemicals which comprises incorporating therein the sodium salt of 30 4:4'-di-(p-amino-benzoyl-amino) stilbene 2:2'-di-sulfonic acid.

13. The method of rendering paper and the like sensitive to ink eradicating chemicals which comprises incorporating therein 4:4'-di-o-chlorobenzoyl-amino stilbene 2:2'-disulfonic acid. 35

14. The method of rendering paper and the like sensitive to ink eradicating chemicals which comprises incorporating therein 4:4'-di-p-methylbenzoyl-amino stilbene 2:2'-disulfonic acid. 40

15. Paper and the like having incorporated therein the sodium salt of 4:4'-di(p-amino-benzoyl-amino) stilbene 2:2'-disulfonic acid.

16. Paper and the like having incorporated 45 therein 4:4'-di-o-chlorobenzoyl-amino stilbene 2:2'-disulfonic acid.

17. Paper and the like having incorporated therein 4:4'-di-p-methylbenzoyl-amino stilbene 2:2'-disulfonic acid. 50

CLIFFORD PAIN.  
JACK AUGUSTUS RADLEY.